

## UNITED STATES PATENT OFFICE

VIKTOR BAUSCH AND KURT FRENZEL, OF BERLIN, GERMANY

TRANSPARENT FOILS OF PAPER, FABRIC, WEBS, AND THE LIKE

No Drawing. Application filed April 3, 1928, Serial No. 267,126, and in Germany April 6, 1927.

Our invention relates to improvements in transparent foils of paper, fabric, webs, and the like and the method of manufacturing the same. More particularly our invention has reference to the method described in the copending application for patent of Bausch, Ser. No. 143,990, filed October 25, 1926, the said method consisting in producing transparent foils by imbuing paper with a medium adapted to render the same transparent. As has been described in the said application for patent, the paper is thoroughly impregnated with a clarifying medium, which clarifying medium is preferably applied in excess on both sides of the paper, and the said excess is maintained during the following treatment of the paper until the finished article is obtained, so that the fibre material is perfectly imbued with the clarifying medium. In the method described in the said application of Bausch resins and similar substances are used as clarifying media, which clarifying media are dissolved in suitable solvents such as alcohol, aceton, and the like. In order to carry out the method in an economical way, it is necessary to regenerate the solvents, for which purpose provision must be made for preventing ignition or explosion of the evaporated solvents. The object of the improvements is to provide a method in which incendiary materials are not used, and which can be carried out at reduced cost, by means of which a better product is obtained, the product being highly transparent and colourless. With this object in view our invention consists in using hydrosols of different characters as clarifying media in lieu of the resins. Suitable clarifying media are the hydrosols of all the colloids the hydrosols of which are capable, when drying, to form more or less clear foils, such for example as albumin, animal glue, carrageen moss, further substances of the character of sugar, such as starch, dextrin, and the like. Further, viscose (cellulose-xanthogenate and cellulose-thiocarbonate) may be used, or thiocarbonate or xanthogenate of other carbohydrates such as starch-xanthogenate, may be used. For example a 30% solution of gelatin has been found to be useful as a clarifying medium. A solution of gelatin or animal glue of this high concentration is very viscous, and it is difficult thoroughly to impregnate the paper by means of such a viscous solution. By adding aliphatic alcohols the viscosity of the solution can be considerably reduced, the ethyl alcohol being particularly suitable for this purpose. The addition of alcohol to the gelatin or animal glue solution may be carried so far that the gelatin or animal glue begins to precipitate. For the same purpose aromatic alcohols soluble in water, for example alcohols of the phenol group, may be added. An addition of carbolic acid is particularly suitable because it improves the transparency of the product. For imparting the desired pliability to the product a softening medium soluble in water is added to the clarifying medium. Suitable softening media are sugar, hygroscopic salts of any character, glycerin, lactic acid, and the like. For hardening the product and improving the transparency thereof we prefer to add formic aldehyde ( $\text{CH}_2\text{O}$ ), urea, and similar substituted aldehydes to the clarifying medium. For hardening the surface of the foil and rendering the same proof against scratching, we expose the foil during or after the drying process to the action of formic aldehyde, for which purpose the foil may be passed through a bath of formalin (a watery solution of formic aldehyde), or treated on one or both faces with formalin vapor. In a modification of the process we add chromium compounds to the hydrosol, or we subject the foil to a subsequent treatment by means of chromic salt solutions, the chromium nitrate  $\text{Cr}(\text{NO}_3)_3$  having been found to be most appropriate as a hardening medium. For imparting, to the foil, a surface which is particularly hard and good we coat the finished foil on both sides with an organosol such as zaponium or acetyl cellulose lacquer.

Transparent foils made by our improved process are optically clear, while chemically and physically they are not homogeneous. Therefore, when drying the same, they tend to form waves, folds and stripes. To prevent

55

60

65

70

75

80

85

90

95

100

the formation of such irregular forms we do not freely suspend the foils at the open air for drying, but we dry the same under tension and on smooth sheet metal, plates, and the like, to which the foils stick while being dried, until the humidity has been removed to a certain degree. Preferably, the tension of the foils is varied in the course of drying, for example by placing the foils on sheet metal and afterwards bending the said sheet metal into cylindric or similar curved form, so that the paper is put under tension. As drying continues, the sheet metal is gradually returned into plane form. By thus subjecting the flexible carrier of the wet foil to different degrees of bending the surface from which the solvent is vaporized is subjected to varying tension, the said varying tension being transmitted to the foil, which therefore can not be formed into waves.

20 The said manner of drying the foil may also be used for imparting a surface appearance of different character to the foil. For example, where a very high transparency is desired a carrier such as sheet metal having a smooth and highly polished surface is used. Where a rough surface is desired we use carriers which are made rough at the surface by corrosion. The said rough carriers are used 25 for example in the manufacture of tracing paper, the result being that the tracing paper readily takes up the ink of the pen or the graphite of the pencil. The tracing paper thus produced has a high transparency.

30 35 The foil may further be dried under tension on sheet metal or cylinders by placing the same on the said carrier alternately with its opposite faces. Thereby both faces are made absolutely smooth and plano-parallel, or one or both faces are made rough and capable of taking up ink.

If it is desired to manufacture a tracing paper the surface of the foil is further treated in order that the graphite of lead-pencils is 40 more readily taken up thereby. For this purpose we apply a coating of a suspension of a suitable powder to one or both faces of the foil, preferably while the foil is wet. Preferably, we use a binding medium which provides 45 a protective colloid for the powder suspended in water, for example a hydrosol such as gelatin or dextrin. When using substances containing gliadin (glutin) as a binding medium and protective colloid for the suspension 50 of powder it is preferred to add thereto a hardening medium such as formalin. The best results have been obtained when using a cold suspension of starch grains as a watery suspension of powder, a suitable composition 55 being 100 gr. cold suspended wheat starch, 2 gr. animal glue, 0.2 gr. alpha-naphthol. The said starch suspension may be sprayed on the wet foil.

In a modification of the process the surface 60 of the foil is coated with an organosol such

as zaponium lacquer containing the powder in suspension, the result being a foil adapted to be written or drawn upon. Other means may be provided for producing a rough surface on the organosol when drying the same. 70

In carrying out the method we proceed in the manner described in detail in the aforesaid application for patent of Bausch. We have found that the foil may be made from certain fabrics such as linen. As has been explained in the said application, it is important that the impregnating medium permeates the whole body of the paper, linen, fabric, or the like, for which reason it is necessary thoroughly to imbue the paper or fabric with the clarifying medium, care being taken that after impregnation and before drying the paper or fabric is coated on both sides with an excess of the clarifying medium. Preferably, the foil consists of a body of paper which has so much of the impregnating medium applied thereto that an additional surface layer of the said medium is provided on both sides of the paper, for which purpose an excess of the impregnating medium is applied to the surfaces of the paper and maintained thereon to the end of the manufacture of the foil. Thereby the surfaces of the foil can be made perfectly plane and parallel to each other, which is necessary for an unimpeded passage of the light rays. Further a film thus prepared is free of minute cavities produced in the interior parts by the drying of the impregnating medium, the parts of the solvent of the impregnating medium escaping when drying the film being replaced by parts of the medium taken from the surface layers. Further, by providing the said surface layers, the 90 hardening of the film by the drying of the impregnating medium is retarded, the said surface layers providing a tight coating retarding evaporation of the solvent and certain softening media added to the impregnated medium. In this respect the property of the outer layers may be improved by properly treating the same, for example by heat, so that the said layers are made sufficiently impermeable to prevent the entire escape of 100 some of the components of the solvent of the impregnating medium and other matter added thereto for softening the film. Therefore the film remains soft and flexible for a considerable length of time even if only a small amount of softening media or no softening media whatever are added to the impregnating medium. The same result may be obtained by coating the foil on both sides with an organosol. 110

When adding suitable hardening media to the impregnating medium, and rapidly heating the surfaces of the film after impregnation thereof the solvent is evaporated mainly on the surfaces of the film, which 120

125

65 130

surfaces are thereby made hard and tight so as to prevent complete evaporation of the solvent within the paper. A film thus prepared has a very hard surface which cannot be spoilt by scratches, and which therefore can be used for a long time.

For accelerating the impregnating operation we first evacuate the paper before passing the same through the impregnating medium, and when passing the previously evacuated paper through the impregnating bath we hold the bath under high pressure.

In the manufacture of the foil we make use of a strong glued paper having a fine and uniform texture. The paper ought to be free of any filling media such as kaolin. We have found that the best results are obtained when using a paper made from rags rather than a paper made from wood cellulose, though our invention is not limited to the treatment of paper made from rags.

In carrying out the process we make use of the apparatus shown and described in the aforesaid application for patent of Bausch.

25 We claim:

1. The herein described method of producing flexible transparent or translucent foils, which consists in thoroughly imbuing paper fabric, or the like with a hydrosol of a colloid, 30 the sol of which is adapted upon drying to produce a more or less transparent foil, and immediately thereafter coating the same on both sides with an excess of such hydrosol, so that the paper, fabric or the like is kept 35 in a state of complete impregnation during and to the end of the drying of the hydrosol.

2. The herein described method of producing flexible transparent or translucent foils, which consists in impregnating paper, fabric or the like with a 30 to 50% solution of 40 gelatin containing an agent adapted to reduce viscosity, maintaining an excess of such hydrosol on the sides of the material being treated so as to keep the same in a state of 45 complete impregnation, and drying the same.

3. The herein described method of producing flexible and transparent foils, which consists in impregnating paper, fabric or the like with a hydrosol of a colloid the sol of which 50 is adapted when drying to produce more or less transparent foils and containing a softening agent adapted to be dissolved in or mixed with water, maintaining an excess of such hydrosol on both sides of the material being 55 treated so as to keep the same in a state of complete impregnation, and drying the same.

4. The herein described method of producing flexible transparent or translucent foils, which consists in impregnating paper, fabric or the like with a hydrosol of a colloid 60 the sol of which is adapted when drying to produce a more or less transparent foil, maintaining an excess of such hydrosol on both sides of the material being treated so as to 65 keep the same in a state of complete impreg-

nation, treating the surfaces of said paper with a hardening medium, and drying the paper, fabric or the like.

5. The herein described method of producing flexible transparent or translucent foils, 70 which consists in impregnating paper, fabric or the like with a hydrosol of a colloid the sol of which is adapted when drying to produce a more or less transparent foil, maintaining an excess of such hydrosol on both sides of the material being treated so as to 75 keep the same in a state of complete impregnation, coating the surfaces of said foil with an organosol, and drying the paper, fabric or the like.

6. The herein described method of producing flexible transparent or translucent foils, 80 which consists in impregnating paper, fabric or the like with a hydrosol of a colloid the sol of which is adapted when drying to produce a more or less transparent foil, and applying to the surface of the impregnated paper a coating of a suspension of an inert powder containing a protective colloid, such coating being capable of drying with a rough 85 surface.

In testimony whereof we have affixed our signatures.

VIKTOR BAUSCH.  
KURT FRENZEL.

95

100

105

110

115

120

125

130